

May 14, 1957

R. H. ATKINSON

2,792,341

PROCESS FOR ELECTRODEPOSITION OF PLATINUM

Filed Dec. 2, 1955



INVENTOR.

RALPH HALL ATKINSON

BY

C. Dr. Deller

ATTORNEY

## 1

2,792,341

## PROCESS FOR ELECTRODEPOSITION OF PLATINUM

Ralph Hall Atkinson, Westfield, N. J., assignor to The International Nickel Company, Inc., New York, N. Y., a corporation of Delaware

Application December 2, 1955, Serial No. 550,632

4 Claims. (Cl. 204—47)

The present invention relates to the electrodeposition of platinum and more particularly to the production of thick, smooth, commercially acceptable electrodeposits of platinum from an acid chloride electrolyte.

It has been well known that thin, adherent electrodeposits of platinum may be obtained by electrolyzing a variety of baths. These thin deposits, as obtained directly from the baths, have been of the order of 0.00001 inch to rarely 0.001 inch in thickness. There are several main classes of baths from which these decorative plates are obtained. Roseleur's bath is an example of one class. This bath contains an aqueous solution of a complex platino phosphate usually modified with suitable buffering and brightening agents. The bath, when used with low cathode current density and when suitably modified, gives bright adherent thin plates which do not require subsequent polishing. Another class of these decorative plating baths is the type using ammoniacal dinitro-diamino platinum as a source of the metal to be deposited. Good throwing power together with bright thin deposits are characteristic of this type of bath. At the same time, the cathode current density may be higher than that used with Roseleur's bath. The third main class of these baths is the alkali platinate type. The platinate is usually buffered and stabilized by the addition of an alkaline oxalate. Under the best conditions, this bath achieves a cathode efficiency, with respect to platinum, of almost 100%. The typical deposits are very bright when thin and the throwing power of the solution is good. Each of the aforementioned baths may be used in a diaphragm cell.

The aforementioned prior platinum plating baths suffer from certain common disadvantages. Thus, the electrolytes are usually unstable, inert salts accumulate during operation, and the cells need constant attention in order to maintain the required concentration of platinum in the electrolyte. None of the prior processes uses a soluble massive anode and, most important, thick, ductile deposits cannot be produced directly from the baths. By using a procedure consisting of plating a thin layer of metal, followed by scratch brushing or polishing the deposit, and then repeating the process as often as required, a thick smooth deposit may be built up. Without this procedure thick deposits are uneven and undesirably crystalline in nature. However, when such repetition procedures are employed, the resulting thick deposits are usually not ductile enough to withstand cold working without cracking.

There have been references to the deposition of platinum from acid chloride media. Generally, only color and adherence were used as criteria for determining whether or not the deposits were satisfactory. One advantage of the acid chloride baths is that under the proper conditions the electrolyte is corrosive to massive platinum. When properly employed, this effect may be used to advantage by providing a soluble anode process. This eliminates the necessity for frequent adjustment of the

## 2

metal concentration in the electrolyte. However, the metal which is deposited under the appropriate conditions for the solution of the anode is, according to the prior art, grossly crystalline or blistered. Kushner (Metal Industry, 1939, page 131) declares that deposits from acid chloride baths are spongy, dark or non-adherent. To my knowledge, no satisfactory ductile platinum electrodeposits have been obtained when using the acid chloride bath under conditions which will efficiently corrode massive platinum anodes.

Although attempts were made to overcome the foregoing difficulties and other disadvantages, none, as far as I am aware, was entirely successful when carried into practice commercially on an industrial scale.

It has now been discovered that thick, smooth, adherent electrodeposits of platinum may be obtained by specially controlling the process when using an electrolyte containing a high concentration of hydrochloric acid.

It is an object of the present invention to provide a process by means of which thick, smooth electrodeposits of platinum may be directly produced in a single plating operation.

Another object of the invention is to provide a process by means of which thick, smooth, ductile electrodeposits of platinum may be made without intermediate brushing or polishing operations.

The invention also contemplates providing a process utilizing a stable bath suitable for the production of thick, smooth, ductile electrodeposits of platinum wherein the concentration of the platinum in the electrolyte will remain within operating specifications.

It is a further object of the invention to provide a process using a stable acid chloride bath from which platinum may be deposited in a form suitable for mechanical working without a prior annealing step.

Other objects and advantages will become apparent from the following description taken in conjunction with the accompanying drawing which shows a special relationship between the concentration of hydrogen chloride in the electrolyte and the rate of deposition of the metal on the cathode which is required according to the present invention in order to obtain the results contemplated by the invention, including electrodeposits of platinum free from cracks as plated.

Generally speaking, the present invention contemplates a process for the production of thick, smooth electrodeposits of platinum from an aqueous bath which contains in solution between about 180 and about 300 grams per liter (g. p. l.) of hydrogen chloride and between about 10 and about 50 g. p. l. of platinum. Platinum is present in the bath chiefly in the form of the complex anion  $\text{PtCl}_6^{4-}$  with small amounts of  $\text{PtCl}_4^{2-}$  being usually co-present. Metal is electrodeposited at a cathode while the bath is maintained at temperatures between about 45° C. and about 90° C. It has unexpectedly been discovered that there is a relationship between the desired physical characteristics of the deposit and a combination of the factors of rate of deposition of metal on the cathode and the concentration of hydrogen chloride in the bath. The accompanying drawing depicts this relationship and shows the particular combinations of rate of deposition and concentration of hydrogen chloride which are applicable to this invention when the bath is maintained within the proper temperature range. When deposits are made under the conditions represented by the area FGHEF bounded by lines FGHE and FE in the accompanying drawing, these deposits are smooth and adherent when appreciable thicknesses are attained and are free from cracks in the as-plated condition. Deposits which are made under the conditions represented by the more restricted area ABCDEA bounded by the lines

ABCDE and AE in the drawing will have the additional feature of being sufficiently ductile in the as-plated condition to withstand appreciable cold working without cracking or separating from the base metal. On the other hand, metal deposited under conditions represented by the areas outside the aforementioned areas of the drawing will be rough, spongy, semiburnt or cracked as plated. For example, if ductility is not an important consideration, thick, smooth adherent deposits of platinum may be obtained with a minimum rate of deposition about  $0.26 \times 10^{-3}$  inch per hour when the hydrogen chloride concentration of the bath is 300 g. p. l. If the concentration of hydrogen chloride is lowered to about 260 g. p. l., the minimum rate of deposition with which thick, smooth adherent deposits may be obtained is about  $0.38 \times 10^{-3}$  inch per hour. Again, if the concentration of hydrogen chloride is lowered still further, to say 180 g. p. l., then a minimum rate of deposition of about  $0.59 \times 10^{-3}$  inch per hour is necessary in order to obtain thick, smooth adherent deposits. At all of these aforementioned concentrations of hydrogen chloride, the maximum rate of deposition with which one can obtain thick, smooth adherent deposits is about  $1.00 \times 10^{-3}$  inch per hour.

Table I illustrates the permissive maximum and minimum values for the rate of deposition which may be used at selected concentrations of hydrogen chloride if one desires to obtain deposits which are not only thick, smooth and adherent but are also ductile.

TABLE I

| Cone. of Hydrogen Chloride in g./l. | Minimum Rate of Dep. in $\text{inch} \times 10^{-3}/\text{hr.}$ | Maximum Rate of Dep. in $\text{inch} \times 10^{-3}/\text{hr.}$ |
|-------------------------------------|-----------------------------------------------------------------|-----------------------------------------------------------------|
| 300                                 | 0.30                                                            | 1.00                                                            |
| 280                                 | 0.36                                                            | 0.96                                                            |
| 260                                 | 0.46                                                            | 0.93                                                            |
| 240                                 | 0.57                                                            | 0.90                                                            |
| 220                                 | 0.68                                                            | 0.84                                                            |
| 215                                 | 0.76                                                            | 0.76                                                            |

It must be noted that the factor of rate of deposition is not equivalent to the cathode current density which is the usual criterion of the electrodepositing art. There is no simple relationship between these two factors when depositing platinum metal from the electrolyte contemplated in this invention. When an article or a series of similar articles are to be plated under a particular set of conditions (e. g., bath composition, temperature, circulation, electrode separation, potential, etc.), the proper rate of deposition must be initially determined by measurement of the change in thickness of the deposit with respect to time. When the proper rate of deposition of metal is obtained in accordance with the invention, the rate may then be maintained by control of the particular conditions (e. g., bath composition, temperature, circulation, electrode spacing, potential, cathode current density or its equivalent cathode current, etc.). Any change in the selected conditions will usually affect the rate of deposition and necessitate another determination of the rate of deposition or a prior determination of the influence of the change upon the rate of deposition.

The cell may be constructed of any material resistant to corrosion by the electrolyte. It may be of a diaphragm or a non-diaphragm type. The diaphragm may be of the usual type and, as those skilled in the art know, it must be resistant to the action of the electrolyte but must permit the passage of the electrical current. It is within the scope of the invention to use either soluble platinum metal anodes or insoluble anodes made from material inert to the action of the electrolyte (e. g., rhodium). When a diaphragm cell is used with soluble platinum anodes, the concentration of platinum metal in the catholyte may be kept within the proper working range by re-

plenishment thereof either from the anolyte or from some external source. In the absence of the diaphragm, the concentration of platinum metal in the electrolyte will remain reasonably uniform due to the similar rates of solution of the anode and deposition of metal on the cathode which are achieved in employing the bath contemplated in accordance with the invention. Only infrequent additions of hydrogen chloride and water are then necessary to replace incidental losses from evaporation and the like.

As was mentioned hereinbefore, the bath from which the metal is deposited is an aqueous acid chloride-chloroplatinic bath which must contain in solution between about 10 and about 50 g. p. l. of platinum. Ordinarily, the platinum is added to the bath initially in the form of chloroplatinic acid. If platinum metal is used as an anode, the concentration of the platinum will be maintained substantially constant during the plating operation due to solution of the metal from the anode. The initial addition of platinum in the form of chloroplatinic acid is recommended because of the convenience of the preparation of this compound. However, if one wishes, the platinum may be added in any form which will produce a solution which is free from materials which will have a detrimental effect on the bath. For convenience's sake, these materials are called subversive materials.

There are several different kinds of these subversive materials, e. g., strong oxidizing and reducing agents should be absent from the bath. The platinum should be predominately in the valence state of four with the ratio of platinic to platinous ions being greater than about twenty to one. Additions of strong reducing agents, particularly organic matter, would tend to decrease this ratio. On the other hand, an excess of strong oxidizing agents will tend to reduce the cathode efficiency. Metals which will hydrolyze in high concentrations of hydrochloric acid, (e. g., titanium, zirconium, etc.), should be absent from the bath because the hydrolysis products of these metal ions may be insoluble substances, colloidal in nature, which would tend to co-deposit with the platinum thus impairing the adherence, continuity and ductility of the deposit. Tungsten and molybdenum should be absent from the bath. These metals represent a class of metallic elements which will form insoluble acids in strongly acidified solutions, e. g., tungstic and molybdic acids. Potassium, ammonium, cesium, rubidium, etc., ions should be substantially absent from the bath because of the well known tendency of these materials to cause the precipitation of platinum as the chloroplatinate, e. g., potassium chloroplatinate. Metals which may co-deposit under the process conditions should be absent from the bath in appreciable quantities. For example, nickel, iron, copper, silver, gold etc., should be absent. It must be understood, however, that impurities normally associated with commercial platinum in quantities normally occurring in commercial grades of platinum do not have any noticeable effect on the character of the deposits.

In view of the foregoing remarks, platinum may be added to the bath not only in the preferred form of chloroplatinic acid but also in the form of any one or a plurality of compounds including sodium chloroplatinate, lithium chloroplatinate, alkaline earth chloroplatinates, hydrated platinic oxide and mixtures of chloroplatinic acid and chloroplatinous acid containing less than about 5% of chloroplatinous acid. When platinum is added to the bath in any of the forms noted herein, it is obvious that there is necessarily added a stoichiometrical amount of the ions associated therewith in the compound. For the purpose of this invention, these associated ions are inert when present in amounts up to about 50 g. p. l. Inert soluble salts should not be allowed to accumulate in the bath. Therefore, it is preferable that platinum compounds which will introduce these inert salts be used only for the initial addition of

platinum to the bath. In addition to the inert substances mentioned in connection with the addition of platinum, the bath may tolerate up to about 50 g. p. l. in the aggregate of inert ingredients, (e. g., the soluble sulfates and acetates of sodium, lithium, alkaline earth metals, magnesium, aluminum, etc.). Included in these inert ingredients and in the aggregate permissive upper limits of concentration are free sulfuric and acetic acids. As far as is known, the addition of moderate amounts, e. g., up to about 50 g. p. l. in the aggregate, of these soluble substances does not effect the working characteristics of the bath as contemplated in this invention. In general, it should be stated that it is preferred to avoid the addition of substantial amounts of anions other than chloride and chloroplatinic because of the complex chemical reactions which may occur in mixtures of this type.

The electrolyte which is employed in accordance with the invention is corrosive to many base metals, such as iron, copper, nickel, zinc, silver, etc. When it is desired to plate on such base metals, they should be given a preliminary strike of a resistant noble metal from a suitable high pH bath in which the concentration of the noble metal ion is low. Satisfactory strike deposits include gold, platinum, palladium or rhodium. Those skilled in the art will recognize that any one of a number of baths designed to deposit these metals may be used. Particular attention should be paid to the surface preparation of the cathode prior to plating these strikes in order to obtain optimum adherence of the strike. The strike should be of such a thickness as to effectively reduce the corrosion rate even in the absence of cathodic protection.

In carrying the invention into practice, it is desirable to maintain the conditions of electrodepositing within the ranges in Table II always keeping in mind that the factors of rate of deposition and concentration of hydrogen chloride must be related to each other as shown in the drawing.

TABLE II

|                                              | Range      |            |
|----------------------------------------------|------------|------------|
|                                              | Broad      | Preferred  |
| Platinum in Bath, grams per liter.           | 10 to 50   | 15 to 25   |
| Hydrogen chloride, grams per liter.          | 180 to 300 | 240 to 260 |
| Rate of Deposition, in./hr. $\times 10^{-3}$ | 0.3 to 1.0 | 0.6 to 0.8 |
| Temperature, °C.                             | 45 to 90   | 65 to 75   |

The rate of circulation during deposition should be low and uniform. Because of the high concentration of hydrochloric acid, the resistance of the bath is low and this resistance is not effected to any great extent by variations in electrode spacing or concentration of platinum. The low resistance of the bath, however, necessitates that the external circuit be controlled very closely so that the cathode current density will be suitable for the particular rate of deposition to be employed.

For the purpose of giving those skilled in the art a better understanding of the invention, the following illustrative examples are given:

## Example I

A plating solution was prepared containing 4 parts by weight of platinum as chloroplatinic acid, 150 parts by weight of concentrated hydrochloric acid and 76 parts by weight of distilled water. The concentration of hydrogen chloride in this electrolyte was about 260 g. p. l. and the platinum concentration was about 20 g. p. l. The electrolyte was placed in a glass container, center portion of the bottom of which was heated, and the temperature was brought to and maintained at 70° C. The cathode was a pure platinum wire 2 inches in length and 0.044 inch in diameter which had been previously cleaned with alkaline cleaning solution and then rinsed thoroughly with distilled water.

70

75

The anodes were two strips of pure platinum, each 5 inches by 0.5 inch by 0.010 inch in dimension with about 1.75 inches immersed in the electrolyte. A potential was applied to the system in order to effect a rate of deposition approximating  $0.5 \times 10^{-3}$  in./hr. The current which was used was 0.055 ampere (amp.), giving a cathode current density of 3.1 amperes per square decimeter (amp./dm.<sup>2</sup>). After one hour it was determined that the metal deposited was  $0.5 \times 10^{-3}$  inch thick and was smooth, adherent and gray in color. A second deposit from the same bath on the same cathode was made with a rate of deposition of about  $0.7 \times 10^{-3}$  in./hr. using a current of 0.060 amp., the cathode current density being 3.4 amp./dm.<sup>2</sup>. At the end of the second hour, the deposit had increased in thickness to  $1.2 \times 10^{-3}$  inch. The entire deposit was smooth, adherent and gray in color and was ductile as indicated by a cold rolling test with 20% cold reduction as the criterion. The deposit, as plated, had an average Knoop Hardness Number (K. H. N.) of 220 using a 25 gram load. The plating solution was stable and had an effective life of at least 57 plating hours with only infrequent additions of hydrochloric acid and water necessary to replace losses due to evaporation.

## Example II

A bath with the same hydrogen chloride concentration as in Example I and having a concentration of 21.8 g. p. l. of platinum as chloroplatinic acid was used to deposit platinum on a platinum strip cathode measuring 1 inch by 0.25 inch by 0.010 inch. Anodes similar to those in Example I were also used. Using a rate of deposition of about  $0.6 \times 10^{-3}$  in./hr. metal was electrodeposited and after six hours at an operating temperature of 70° C. a deposit  $3.63 \times 10^{-3}$  inch thick was obtained. The current used was 0.080 amp. and the cathode current density was 2.4 amp./dm.<sup>2</sup>. The resulting deposit was uniform, ductile, adherent and had an average hardness of 214 K. H. N. with a 25 gram load.

## Example III

A glass container was separated into anodic and cathodic compartments through the use of a porous porcelain diaphragm. A solution similar to that used in Example I was placed in the cathodic compartment. A hydrochloric acid electrolyte was used as the anolyte. The anodes and cathode were similar to those used in Example I and the operating temperature was 70° C. A rate of deposition of approximately  $0.7 \times 10^{-3}$  in./hr. was established and after one hour,  $0.67 \times 10^{-3}$  inch of metal was deposited using a current of 0.045 amp. and a current density of 2.6 amps./dm.<sup>2</sup>. The deposit was light gray in color, smooth, adherent and free from cracks as plated. A further deposit at approximately the same rate of deposition was made on the same cathode, and after another hour the deposit was found to have increased in thickness to  $1.35 \times 10^{-3}$  inch. A current of 0.040 amp. with a cathode current density of 2.3 amps./dm.<sup>2</sup> was used for this second hour. The total deposit was smooth and ductile and had an average hardness of 194 K. H. N. with a 25 gram load. Chemical analysis of the catholyte revealed that its platinum content was reduced from 23 down to 15 g. p. l. in the course of two hours' plating in the absence of replenishment.

## Example IV

A plating solution was prepared having a platinum concentration of 22 g. p. l. and a hydrogen chloride concentration of 219 g. p. l. It was placed in a glass container similar to the one used in Example I and heated to about 70° C. in the same manner as in Example I. The cathode was a platinum wire having the same dimensions as the cathode in Example I. This cathode was previously cleaned in alkaline cleaning solution and thoroughly rinsed in distilled water. The anodes were the same as used in Example I. A potential was ap-

plied to the system in order to effect a rate of deposition approximating  $0.9 \times 10^{-3}$  in./hr. The current which was used was 0.063 amp. giving a cathode current density of 3.5 amps./dm.<sup>2</sup>. After one hour, it was determined that the metal deposited was  $0.88 \times 10^{-3}$  inch thick and was a smooth gray mat showing no cracks as plated when examined under the microscope. The deposit had an average Knoop Hardness Number with a 25 gram load of about 274. It was found to be brittle when cold rolled for a 20% cold reduction.

*Example V*

A plating solution was prepared having a platinum concentration of 23.6 g. p. l. and a hydrogen chloride concentration of about 260 g. p. l. The cathodes, anodes and cell were similar to those used in Example I. A temperature of about 45° C. was attained and maintained. A potential was applied to the system in order to effect a rate of deposition approximating  $0.5 \times 10^{-3}$  in./hr. After one hour, it was determined that the metal deposited was  $0.49 \times 10^{-3}$  inch thick. The current employed was 0.035 amp. and the cathode current density was 2.0 amps./dm.<sup>2</sup>. Visual examination revealed that the plate was a light gray mat. On microscopic examination the plate was found to be free from cracks. The average Knoop Hardness Number with a 25 gram load was 241 and the plate was found to be ductile upon a 20% cold rolling reduction.

The following test was conducted to illustrate the effect of using a rate of deposition which, when plotted against the hydrogen chloride concentration, results in a point that lies outside the area FGHEF in the drawing. In conducting this test, a plating solution was prepared containing 222 g. p. l. of hydrogen chloride and 22 g. p. l. of platinum. The plating run was made at a temperature of 70° C. for three hours with a current of 0.045 amp. and a cathode current density of 2.5 amps./dm.<sup>2</sup>. The rate of deposition was  $0.27 \times 10^{-3}$  in./hr. Upon superficial examination, the deposit  $0.80 \times 10^{-3}$  inch thick was found to be smooth, dark gray with slight sheen, hard and brittle. Microexamination revealed that the deposit was cracked as plated.

The data set forth in Table III illustrate the fact that cathode current density and rate of deposition are not equivalents when depositing from the acid chloroplatinate baths at a standard temperature (70° C.).

TABLE III

| Cathode C. D.<br>amps./dm. <sup>2</sup> | Rate of Dep.<br>$10^{-3}$ in./hr. |
|-----------------------------------------|-----------------------------------|
| 3.5                                     | 0.88                              |
| 3.4                                     | 0.70                              |
| 3.1                                     | 0.50                              |
| 2.6                                     | 0.67                              |
| 2.5                                     | 0.27                              |
| 2.4                                     | 0.61                              |
| 2.3                                     | 0.68                              |

The present invention is particularly applicable to the production of electroplates of platinum for both protective and decorative purposes. As a result of using this process, the plated bodies will withstand the corrosion of any agents to which platinum itself is resistant. Ductile deposits of platinum may also be used in the electro-forming and electrorefining arts, giving the advantage of ductility inherent in the deposits without the necessity of annealing or other subsequent heat treatment. Smoothness of deposit usually is an important factor in these arts.

It is to be observed that the present invention provides a process for the production of thick, smooth ductile electrodeposits of platinum. In carrying out the invention, deposits up to about 0.02 inch in thickness are readily obtained. The process involves electrolyzing the bath under stated conditions of rate of metal deposition correlated to hydrogen chloride concentration. The essential ingredients of the bath are an aqueous solution of hydrogen chloride and a source of chloroplatinic ion. The platinum in this bath is associated with chlorine such that the ratio of platinum in the chloroplatinic form to platinum in the chloroplatinous form is at least about 20:1. The balance of the bath is essentially water. However, the inclusion of 0 to about 50 g. p. l. in the aggregate of soluble non-subversive inert substances, e. g., sodium salts, lithium salts, sulfuric acid, acetic acid, alkaline earth metal salts, etc. is contemplated within the meaning of the term "balance essentially."

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. A process for the production of thick, smooth, adherent electrodeposits of platinum free from cracks in the as-plated condition which comprises establishing an aqueous acid chloride-chloroplatinate bath containing in solution about 180 to about 300 grams per liter of hydrogen chloride, about 10 to about 50 grams per liter of platinum to provide a source of chloroplatinic ion, the balance being essentially water and electrodepositing platinum from said bath while maintaining the bath at a temperature between about 45° C. and about 90° C. at such a rate of deposition that the rate of deposition of the metal on the cathode when plotted against the concentration of hydrogen chloride in the bath will be represented by a point lying within the area FGHEF in the accompanying drawing.

2. A process as set forth and described in claim 1 wherein the bath is maintained at a temperature between about 65° C. and about 75° C.

3. A process for the production of thick, smooth adherent, ductile electrodeposits of platinum free from cracks in the as-plated condition which comprises establishing an aqueous acid chloride-chloroplatinate bath containing in solution about 215 to about 300 grams per liter of hydrogen chloride, about 10 to about 50 grams per liter of platinum to provide a source of chloroplatinic ion, the balance being essentially water and electrodepositing platinum from said bath while maintaining the bath at a temperature between about 45° C. and about 90° C. at such a rate of deposition that the rate of deposition of the metal on the cathode when plotted against the concentration of hydrogen chloride in the bath will be represented by a point lying within the area ABCDEA in the accompanying drawing.

4. A process as set forth and described in claim 3 wherein the bath is maintained at a temperature between about 65° C. and about 75° C.

References Cited in the file of this patent

Kishner: Metal Industry, volume 37 (1939), page 131.